

1

3,004,312

## PROCESS OF SHELL MOLDING

Charles F. Froberger, Oak Park, Mich., assignor to General Motors Corporation, Detroit, Mich., a corporation of Delaware

No Drawing. Filed June 25, 1953, Ser. No. 364,202

4 Claims. (Cl. 22—193)

This invention relates to improvements in shell molding and more particularly to an improved method of forming shell molds for use in the precision casting of metals.

Recently developed techniques in foundry practice employ thin-walled dispensable molds and cores composed of sand and thermosetting binders. These procedures, generally referred to as "shell molding" processes, are particularly suited for the production of precision castings of a wide variety of metals.

Essentially the shell molding process consists of employing a heat-hardenable plastic or resin as a binder for the sand grains to form rigid molds having high gas permeability, good surface smoothness and dimensional stability. The molding material, generally a dry mixture of a major proportion of silica sand and a minor proportion of a thermosetting binder, is used in a powdered form with no water being added. Phenol-formaldehyde, phenol-furfural, melamine-formaldehyde and urea-formaldehyde resins are typical examples of the type of thermosetting binders preferably used. It is desirable that the sand employed be free of metal oxides, clay, moisture and organic matter.

These sand-resin molds are prepared by allowing the dry mixture of sand and powdered resin to come into contact with a hot metal pattern for a short period of time. A layer of the mix adheres to the metal pattern surface due to the heating of the resin which entraps the sand with which it is intimately mixed, thereby accurately reproducing pattern details. The half patterns, gates and runners are usually all permanently fixed on metal plates. Metal patterns must be used because they are subjected to elevated temperatures. Pattern temperatures in the range between 250° F. and 450° F. are typical, but under certain conditions temperatures up to about 800° F. may be advantageously employed. The pattern temperature and the length of time the molding material is allowed to remain in contact with the hot pattern surface determine the resulting thickness of the mold. Mold build-up times generally range from a few seconds to approximately two minutes, depending upon the particular application.

After this short time interval, any excess or unbonded sand and resin are removed, and the closely adhering sand-resin layer is cured, preferably by heating to a temperature within the range of about 300° F. to 1500° F. for a short period of time, usually from a few seconds to approximately five minutes, while in contact with the metal pattern. This baking operation results in the conversion of the resinous material to a hard, insoluble binder which securely bonds the sand grains together. After the removal of the pattern and mold from the curing oven, the mold is stripped from the pattern. The completed molds are, in effect, thin shells which possess sufficient strength and stiffness to make them suitable for many casting operations.

One of the primary reasons for the relatively restricted use of the shell molding process up to the present time has been the comparatively high cost of the organic binder. Inasmuch as the sand-resin mix normally contains up to about 15% by weight of a thermosetting resin binder, the cost of the binder has been a substantial item of expense when this process is employed. This is particularly true in applications which require the inclusion of a finely comminuted refractory material, such

2

as silica flour or powdered spent catalyst material, in the molding mix since such a mixture necessitates the use of an exceptionally high binder content. The employment of a mix containing such a fine refractory facing is especially desirable in casting steel or other high melting metals by the shell molding process, a procedure which previously has been impracticable.

Conventionally, a powdered thermosetting resin and a curing agent are mixed with the desired quantity of a suitable refractory filler material, and the dry mixture is applied to the hot pattern without further preparation. Although the use of such a molding mix generally provides satisfactory shell molds in most respects, it also results in an undesirable residue build-up on the pattern. Moreover, the shell molds heretofore used generally have proved to be somewhat brittle and not sufficiently strong or resilient to provide optimum results in all instances.

Accordingly, a principal object of the present invention is to provide an improved shell mold and a method of preparing the same in which forming of the mold shell does not result in a pattern build-up. The elimination of this build-up in turn permits the same pattern to be used over a greatly extended period of time without the necessity of removing the residue therefrom in order to accurately reproduce pattern details.

A further object of my invention is to provide an improved shell mold and organic binder therefor which are appreciably less expensive than those generally heretofore used. A still further object of this invention is to provide a process for forming shell molds in which the amount of the relatively costly thermosetting resin binder may be substantially reduced, amounts in the order of approximately 2% by weight being all that is necessary for many applications.

The above and other objects are attained in accordance with my invention by the use of sand or other suitable comminuted refractory material having a substantial portion of its particles coated with an improved binder to form relatively inexpensive shell molds without building up a residue layer on the patterns. The improved organic binder which is used to coat the sand particles comprises a mixture of novolak and a thermoplastic resinous material derived from wood. A small amount of a curing agent is also added in the molding mix to promote the proper setting of the binder upon subsequent contact of the molding mix with the hot pattern.

Certain of the resoles may be included in the binder as a substitute for a portion of all of the novolak provided they may be conveniently melted without setting. Generally, however, it is preferred to use only a small percentage of resole in place of novolak, and excellent results appear to be obtained when resole is omitted entirely. In all instances, of course, it is necessary that the binder mixture sets, at least partially, at the temperature of the hot pattern.

The thermoplastic resinous material derived from wood may be blended with the novolak either by means of solvent blending or solid fusion. The novolak provides the mold with smooth casting-defining surfaces and high strength, while the thermoplastic resinous material is employed as a copolymerizable substance to provide improved bonding together of the sand particles as well as to improve the strength of the mold.

During the formation of a shell mold according to the present invention, an improved casting-defining mold surface results from the co-condensation or copolymerization of the thermoplastic resinous material and the novolak to form a substantially completely thermoset product with a relatively small amount of expensive binder constituents. The novolak preferably is partially polymerized when mixed with the thermoplastic resin-

ous material so that only a short baking period is required to cure the binder mixture.

It will be understood that the term "mold," as used herein, is applied in its generic sense to mean a casting form which includes both molds and cores, this invention in no manner being limited to the former. Similarly, unless otherwise indicated, the word "pattern" is used herein as including both mold patterns and core boxes.

Other objects and advantages of this invention will more fully appear from the following detailed description of preferred methods of employing my novel binder to form an inexpensive shell mold which eliminates the formation of the undesirable residue build-up on the pattern surfaces.

In preparing the improved organic binder for the shell mold, the novolak and/or resole may be first intimately mixed with the thermoplastic resinous material derived from wood. These binder constituents are then blended with the sand while in a molten condition to effectively coat the surfaces of the individual sand grains. A small but effective amount of an accelerator or co-condensating agent, such as hexamethylene tetramine or paraformaldehyde, is then added to the molding mix to promote the curing of the principal binder constituents when the molding mix is later placed into contact with the hot pattern.

Normally the curing agent should not be present in an amount greater than approximately 25% by weight of the total binder. If an excess of curing agent is employed, thermal stresses are set up in the mold on pouring of the molten casting metal, and cracking of the mold occurs. Hence it is preferred to add the curing agent in an amount between approximately 8% and 15% of the weight of the binder.

I have found that, in order to properly benefit from the present invention, the lignin-type resin should constitute at least approximately 25% by weight of the binder. Greater amounts, in some cases up to about 80% by weight, also may be used. In the formation of shell molds suitable for many casting operations I have found that superior results are obtained if the organic binder contains about 40% to 60% by weight of the lignin-type resin, approximately 50% by weight being preferred at present.

The term "thermoplastic material derived from wood," hereinafter used as descriptive of the thermoplastic material in accordance with the invention, is intended to include various wood derivative resinous materials in which the molecules contain both methoxyl and hydroxyl groups. Such materials may be obtained from a variety of wood products including sawdust, wood chips, etc., by physical and/or chemical treatment. Illustrative of one type of thermoplastic resinous material is a substantially gasoline-insoluble resinous material obtained by extracting a resinous wood with a coal tar hydrocarbon, removing said hydrocarbon by evaporation, leaving a residue comprising a mixture of wood rosin and thermoplastic resinous material, extracting the rosin with a petroleum hydrocarbon, leaving a thermoplastic resinous material, hereinafter referred to as a gasoline-insoluble wood resin. Such a material is currently available commercially as "Vinsol" resin, a product of the Hercules Powder Company.

In practice, the amount of the organic binding mixture of the present invention to be employed in a particular shell molding operation may be varied, although in general it is desirable to employ a relatively small amount of binder to reduce the cost of the molds. When employing organic binders of the present invention I have found that in many cases as little as approximately 2% by weight of the total binder may be used. The maximum amount of binder to be employed generally is determined by cost considerations, although in most cases superior results are obtained if the amount of the binder is not permitted to exceed about 15% of the total weight.

of the molding mix. Hence, in order to obtain satisfactory casting at a reasonable cost, a binder content between 3% and 7% is preferred.

Ordinary sand or other comminuted refractory filler material's, such as zirconium silicate sands and flours, are appropriate for use in practicing the present invention and normally constitute between 85% and 98% of the weight of the molding mix. In most cases it is desirable to employ a refractory material having an American Foundryman's Society fineness number within the range of about 25 to 180. At present I prefer to employ a refractory material having an AFS fineness number within the range of 50 to 125.

In many instances it is desirable to also employ fine refractory materials or powders, such as silica flour or powdered spent catalyst, etc. as fines to provide a better mold facing surface. In practice, amounts of such facing materials within the range of about 2% to 20% by weight are used in many cases to provide a more heat-resistant mold surface. Thus I have obtained very beneficial results in the casting of steel by a shell molding process when the mixture forming the shell mold is composed essentially of about 75% to 95% by weight of dry sand, about 2% to 20% by weight of silica flour or other finely divided refractory material, and about 5% to 15% of the organic binder.

In the formation of a shell mold of the present type, which is characterized by the elimination of pattern build-up and excellent casting-defining surfaces, the novolak may be first dissolved in a suitable solvent, such as methyl-ethyl ketone or a mixture of toluene and methyl alcohol. After the novolak is dissolved in the solvent, the thermoplastic material derived from wood is added to the solution and also dissolved therein. Normally as much of these constituents are dissolved in a given amount of solvent as feasible. In practice, when a sufficient amount of the thermoplastic material derived from wood has been added so that this resin and the novolak constitute at least approximately 80% by weight of the total mixture or solution, the blend of these constituents is heated to a temperature at which it flows freely before it is mixed with the sand. Generally a temperature of at least 150° F. is therefore desirable. Of course, the solvent and the binder constituents may be initially heated and maintained at this elevated temperature while the latter are being dissolved in the solvent.

The sand is also preferably heated to prevent the organic binder constituents from cooling too rapidly and to insure the proper coating of the binder on the sand grains. Hence, I have found it advisable to heat the sand to a temperature of approximately 600° F. and then to permit the sand to cool to approximately 400° F. before the binder-solvent is introduced. In general, satisfactory results are provided if the temperature of the sand is between 300° F. and 500° F. when the binder is added. During the mulling operation in which the binder is completely blended with the sand, the mixture cools and the solvent evaporates, leaving a coating of the mixture of the novolak and the lignin-type resin on the sand particles.

When the temperature of the coated sand has dropped to a temperature which is sufficiently low to preclude setting or curing of the binder upon addition of the curing agent, the latter is added to the molding mix. I have found a temperature between approximately 100° F. and 150° F. to be satisfactory in this respect. Likewise, the molding mix may be easily milled at this temperature. The mulling operation is continued, of course, until the curing agent is thoroughly mixed with the coated sand grains.

Although excellent results are obtained using the above-described method of coating the sand particles with the novolak and thermoplastic material derived from wood, it is not necessary to introduce the binder to the sand by

means of a solvent. If the sand is maintained at a sufficiently high temperature, it is possible to add these powdered materials directly to the hot sand and to use the heat in the sand to melt and distribute the binder. The flow characteristics of the lignin-type resin and novolak mixture are such as to permit satisfactory coating of the sand particles under these conditions. For example, the solvent may be omitted and the novolak and thermoplastic material derived from wood first can be melted together, or separately melted and blended. Then this binder mixture may be permitted to cool and crushed to a powder form before being added directly to the hot sand. Likewise, it is also possible to separately or simultaneously mix the thermoplastic material derived from wood and novolak with the hot sand in powder form, or these two powders may be pre-mixed and then thoroughly blended with the sand which is preferably maintained at the aforementioned elevated temperatures. Alternatively, the novolak and the thermoplastic material derived from wood can be melted and added, either simultaneously or successively to the heated sand while in a liquid condition. If desired, of course, these liquid binder constituents may be blended together, either as liquids or powders, before being introduced to the sand as a hot liquid.

After the particles of sand or other refractory material are coated with the organic binder in the above-described manner, the resulting mixture is placed in contact with the surface of a heated pattern having a temperature of at least approximately 350° F. At temperatures below about 350° F. the thermoplastic material derived from wood will not melt or flow to a sufficient extent to be of any value in strengthening the mold.

To obtain the proper resin flow, the mold mixture should remain in contact with the heated pattern surface for at least 10 seconds with a contact time of between 20 and 35 seconds at the above pattern temperature usually providing highly satisfactory results. In general, there is no maximum pattern contacting time because the mold build-up on the pattern is sufficiently rapid so that heat is quickly conducted from the pattern and soon results in the lowering of the pattern temperature below 350° F. if no further heat is applied to this mold, thus precluding further flowing of the thermoplastic material or burning of the mold. In practice, however, approximately two minutes should be considered as the maximum period the mold should be allowed to contact the hot pattern before removal of the mold-pattern assembly for curing.

The resulting mold must be subsequently baked to complete the cure of the shell mold. The time of curing or baking in most cases should be between about 30 and 120 seconds, a 40 to 90 second cure normally providing optimum results. Of course, the length of the curing period depends on the baking temperature, the higher the curing temperature, the shorter the curing time, and vice versa. Curing temperatures between 350° F. and 1500° F. have proved to be satisfactory although in some cases oven temperatures as high as 1800° F. may be employed. Placing the molded mix into contact with the hot metallic pattern, together with the subsequent baking operation, cures or hardens the binder by causing a copolymerization of the lignin-type resin and the thermosetting resin with the aid of the included small proportion of hexamethylene tetramine, paraformaldehyde or similar curing agent. The sand-resin shell-type mold thus produced has excellent permeability, possesses high transverse strength and exhibits no tendency to cause blowing on the casting when the molten metal is poured.

Shell molds formed in accordance with the above-outlined procedure, while utilizing a relatively small amount of expensive thermosetting resin, thus appreciably reducing the cost, can be employed in the casting of metals to very close dimensional tolerances since the casting-defining surfaces of the mold, while readily permeable to gases, have high strength and smoothness.

These molds have proved to be highly satisfactory at casting metals poured at temperatures as high as 2800° F. and are therefore especially adapted for pouring steel. As indicated above, it is usually desirable to include a minor proportion of a fine refractory filler when casting high-temperature ferrous-base metals. Of course, the above method of forming inexpensive high-strength shell molds permits the precision casting of non-ferrous as well as ferrous metals.

10 On pouring the liquid metal into the mold or core cavity in the usual way, the hot metal, on coming into contact with the mold or core, burns the plastic binder to essentially carbon. The gases which are generated readily escape through the highly permeable sand-resin shell. As a result of this plastic breakdown, the shake-out is easily accomplished.

15 Among the numerous other advantages of this process and the molds produced thereby is the fact that these molds offer very little resistance to the expansion and contraction of the molten metal subsequent to pouring, thus minimizing the danger of formation of cracks or hot tears. The cured shell molds also accurately reproduce pattern details, have no affinity for water, are stable under atmospheric conditions, and may be stored indefinitely.

20 Furthermore, these molds can be produced and processed without dust formation. Moreover, the resultant castings have unusually smooth and clean surfaces, true dimensions, and a minimum of fin at the parting line. The surfaces of these castings are free of residual mold material, thereby eliminating the necessity of shot blasting. This process and the molds formed in accordance therewith can be used to provide castings of extremely thin section due to the unusual smoothness and high gas permeability of the molds.

25 35 It will be understood, of course, that various changes and modifications of the embodiments of the invention described herein may be made by those skilled in the art without departing from the spirit and principles of the invention, the scope of which is defined in the following claims.

I claim:

30 1. A process for forming a smooth-surfaced shell mold without building up a residue layer on a pattern, said process comprising thoroughly mixing a heated comminuted refractory filler with a mold binder comprising novolak and a thermoplastic resinous material obtained by extracting a resinous wood with a coal tar hydrocarbon, removing said hydrocarbon by evaporation, leaving a residue comprising wood rosin and thermoplastic resinous material, and extracting the rosin from said residue with a petroleum hydrocarbon, permitting said sand to cool to thereby cause a coating of the novolak and thermoplastic resinous material to be formed on a substantial portion of the particles of refractory filler, thereafter mixing a small but effective amount of a binder curing agent with the coated sand particles, placing said coated sand particles into contact with a metallic pattern heated to a temperature between 250° F. and 300° F. for at least ten seconds, and thereafter curing 40 the resultant shell mold while in contact with said pattern.

35 2. A method of forming a molding mixture to be applied to a hot pattern for forming a shell mold, said method including thoroughly mixing a heated comminuted refractory filler with a mold binder comprising novolak and a thermoplastic resinous material derived from wood containing both methoxyl and hydroxyl groups, permitting said sand to cool to thereby cause a coating of the novolak and thermoplastic resinous material to be formed on the particles of refractory filler, and thereafter mixing a small but effective amount of a binder curing agent with the refractory filler and binder.

40 3. A method of forming a molding mixture to be applied to a hot pattern for forming a shell mold, said method comprising dissolving in a suitable solvent novol-

lak and a gasoline-insoluble, thermoplastic wood resin containing both methoxyl and hydroxyl groups, intimately mixing the resultant solution with heated sand, thereafter permitting said solvent to evaporate so as to leave a coating of the mixture of the thermoplastic wood resin and novolak on the sand grains, subsequently adding a small but effective amount of a binder curing agent to the coated sand grains, and finally mulling the formed mixture until the curing agent is thoroughly mixed with the coated sand grains.

4. The process of forming a molding mixture to be applied to a hot pattern for forming a shell mold, said process comprising heating sand to a temperature of at least 300° F., melting novolak and a gasoline-insoluble resinous material obtained by extracting a resinous wood with a coal tar hydrocarbon, removing said hydrocarbon by evaporation, leaving a residue comprising wood rosin and thermoplastic resinous material, and extracting the rosin from said residue with a petroleum hydrocarbon, adding these molten materials to the heated sand in an amount constituting between approximately 2% and 15% by weight of the resultant molding mixture, thoroughly mixing said molten materials with said sand to thereby coat the sand particles with said materials, permitting the coated sand particles to cool to a temperature not in 20

excess of approximately 150° F., and thereafter thoroughly mixing a binder curing agent with the coated sand particles in an amount equal to about 8% to 15% of the total weight of the novolak, thermoplastic resinous material and curing agent.

## References Cited in the file of this patent.

## UNITED STATES PATENTS

|    |           |               |               |
|----|-----------|---------------|---------------|
| 10 | 2,101,330 | Delaney       | Dec. 7, 1937  |
|    | 2,405,650 | Hartwig       | Aug. 13, 1946 |
|    | 2,444,413 | Weston        | July 6, 1948  |
|    | 2,491,006 | Grube         | Dec. 13, 1949 |
|    | 2,549,822 | Koonee        | Apr. 24, 1951 |
|    | 2,630,608 | Granath       | Mar. 10, 1953 |
|    | 2,683,296 | Drumm et al.  | July 13, 1954 |
|    | 2,706,188 | Fitkov et al. | Apr. 12, 1955 |
|    | 2,751,650 | Froberger     | June 26, 1956 |

## OTHER REFERENCES

Am. Foundryman, August 1952, pages 42-56.  
The Foundryman, October 1950, pages 162, 164 and 168.  
Steel, December 3, 1951, pages 90 and 92.